

## UNITED STATES PATENT OFFICE

2,236,120

## LUBRICANT FOR INTERNAL COMBUSTION ENGINES

Norbert F. Toussaint, Philadelphia, Hannibal J. R. Gaspari, Blawnox, and Henry A. Ambrose, Penn Township, Allegheny County, Pa., assignors to Gulf Research & Development Company, Pittsburgh, Pa., a corporation of Delaware

No Drawing. Application January 17, 1939,  
Serial No. 251,434

4 Claims. (Cl. 252—35)

Our invention relates to improved lubricants for use in internal combustion engines, such as automotive engines, aviation engines and Diesel-type engines.

5 Progress in the design of internal combustion engines of all kinds tends to impose more and more severe burdens upon lubricants employed therein. The general tendency is always in the direction of higher performance and increased 10 horse-power per unit of weight. This tends to make lubrication more difficult and frequently to introduce entirely new problems into the preparation and selection of lubricants for a particular engine or type of engine. Individual lubricating problems arise with reference to different 15 points in the engine. A satisfactory solution of any one of these individual problems alone is sometimes difficult enough in itself but becomes further complicated when, as is frequently the 20 case, it is found that improvement of a lubricant with respect to one problem may make another problem in the same engine more serious.

Thus, it has been found that a lubricant giving 25 generally good "crankcase performance" in a particular engine may not be entirely satisfactory for lubrication of the cylinder walls, piston and piston rings of the same engine, and vice versa. That is because entirely different physical 30 conditions are encountered in the cylinders than are encountered in the crankcase. Temperatures, rubbing speeds, unit pressures, and other factors vary considerably at different points in any internal combustion engine. Nevertheless the design of internal combustion engines is such that 35 a single lubricant is required, and that lubricant must give satisfactory service under the variety of conditions encountered in each engine.

To illustrate this more fully, a good crankcase lubricant should be as free as possible from 40 sludging tendencies, and its viscosity change over a given temperature variation should be a minimum, i. e. it should have a high viscosity index. Paraffinic petroleum oils, such as those obtained from Pennsylvania crudes, possess these characteristics to a greater extent than do lubricating 45 oils made by ordinary refining methods from less highly paraffinic crudes, such as Coastal and Mid-Continent crudes. During the past decade or so, great strides have been made in refining 50 methods, so that it is now possible to produce from the less highly paraffinic crudes lubricating oils which approach Pennsylvania lubricating oils in general performance characteristics. Even Pennsylvania oils are refined to increase their 55 purity and paraffinicity. One of the best gen-

eral automotive lubricants in use today is made from Pennsylvania crude stock, drastically refined by means of aluminum chloride; the resultant lubricating oil, without any synthetic additions, is approached in value only by some 5 oils which have been carefully refined and then improved by the addition of various and more or less synthetic improvement agents.

In any event, the general crankcase performance of such oils is excellent and they command 10 a justified premium on that account.

Nevertheless, as might be expected, the fact 15 that these oils possess excellent crankcase performance characteristics does not mean that these oils are not susceptible to improvement with respect to performance under special conditions and at particular points in internal combustion engines where the conditions are radically different from those encountered in the crankcase. Moreover, in improving such highly 20 refined oils, with respect to their performance characteristics under such particular conditions, problems are sometimes encountered which, for various reasons, are more difficult to solve than 25 would be true of less highly refined oils.

That has been true, for example, with respect 30 to the corrosion of certain types of corrosion-sensitive metal bearing alloys, of which the so-called "cadmium-silver," "copper-lead" and "cadmium-nickel" bearing alloys constitute examples. In proper engine designs these bearings should give little or no trouble with any oil, but in occasional instances the design of the 35 engine may be such (particularly where excessive bearing temperatures are maintained) that we are confronted with the apparent paradox that the "best" oils do not give the best over-all results and may even be undesirable under particular conditions. It is generally known that 40 the more highly refined oils are, for some reason, occasionally more likely to cause more corrosion of sensitive alloy bearings at high temperatures than is true of the less highly refined oils.

Our invention is not primarily concerned with 45 the solution of the problem of lubricating sensitive metal alloy bearings, and the foregoing is mentioned simply for the purpose of illustrating the complexity of the problem of producing a satisfactory lubricant which, in use, must encounter a considerable variety of specific lubricating conditions.

It might at first be thought that the simple 50 remedy would be to reduce the degree of refining and to go back to cheaper oils. That can be done, however, only by sacrificing general crank- 55

case performance characteristics of the highly refined oils, which is undesirable. And it has been found that this particular problem can be met satisfactorily and without such a sacrifice, 5 by the use of small quantities of addition agents having a specific and beneficial effect upon the particular problem referred to but which do not impair the primary physical characteristics and the general performance characteristics of the 10 lubricant. Obviously, that is the way the problem should be solved.

Our invention is, however, more particularly concerned with the problems encountered in upper cylinder lubrication of internal combustion engines. The difficulties encountered in the cylinders manifest themselves most apparently, from the standpoint of the user, in what is generally known as "ring-sticking." No internal combustion engines of the ordinary type are entirely 15 free from this tendency, but it is encountered more frequently and more seriously in connection with heavy-duty engines, such as Diesel-type and aviation engines. The disadvantages of a lubricant which tends to cause the piston rings 20 to become stuck are too obvious to require discussion. Suffice it to say that a satisfactory lubricant should permit an engine to run at high speed and under high load for a long period of time without any appreciable ring-sticking tendency, other than that attributable to mechanical 25 features of the engine design rather than to any failure on the part of the lubricant.

The problem of ring-sticking is extraordinarily complex. That this would necessarily be the 30 case is evident from the fact that combustion is taking place at or adjacent to the points requiring lubrication. Temperatures tend to be very high, and there is a pronounced tendency for the lubricating oil to be burned or oxidized or otherwise removed from the metallic surfaces in moving contact with each other. Years will probably pass and much intensive research will be done before those in the art are able to specify with any degree of certainty the fundamental cause 35 or causes underlying the "ring-sticking" tendencies and characteristics of petroleum lubricants.

It has been observed that ring-sticking is usually accompanied by the accretion of more or less solid deposits around the rings and on the adjacent metal surfaces being lubricated. These deposits may take the form of carbon, or heavy hydrocarbons (generally referred to as "gum," although not necessarily analogous to the gums 40 formed in cracked gasoline distillates), or they may appear as lacquer-like deposits. These three types of deposits result from various types of chemical actions and are not necessarily interrelated except for the fact that they are solid 45 in character; for that reason their accretion tends to prevent or interfere with normal action of the piston rings. No oils are entirely free from these tendencies, but some oils, for no readily apparent reason, are better than others, and 50 oils which may produce generally equivalent results may actually do so through the mechanism of entirely different chemical reactions.

Thus it has been observed that in the operation 55 of Diesel engines, using lubricants derived from Coastal crudes, ring-sticking tendencies tend to show up more rapidly and more seriously with respect to the bottom piston rings of a particular engine, whereas there is a tendency for the top rings to stick first when the same engine 60 is lubricated with paraffin base oils. It would

appear that the phenomenon is not only connected with temperature but also with the chemical composition of the oil.

On the other hand, a lubricating oil which tends to undergo excessive sludging in the crankcase may give excellent performance characteristics with respect to ring-sticking. Such an oil, even when employed in a heavy-duty Diesel engine, may leave the piston ring assemblages relatively clean and clear. A better oil, however, 5 should give good over-all performance characteristics. It should not be necessary to sacrifice desirable crankcase performance characteristics in order to achieve freedom from ring-sticking and the deposition of gum and lacquer in the 10 upper cylinders.

We have found that in general the deposition of gum in the cylinders is related in some manner to the volatility of the lubricating oil, and that as between two oils of the same viscosity, one 15 of which is a straight distillate (particularly one having a low end boiling point) and the other is a residual oil or a blend containing a residual oil, the latter will be found to cause more gum formation and hence more ring-sticking than 20 will be true of the former. It is not, however, possible to overcome the problem fully by simply employing a distillate oil or selecting an oil 25 of a given volatility.

Others have suggested, prior to our invention, 30 that certain metallic soaps will stabilize petroleum lubricating oils against oxidation, polymerization or a combination thereof, which would ordinarily tend to result in the deposition of carbonaceous material or sludge and in an undesirable change of color. The naphthenates of 35 manganese, cobalt, lead and zinc have all been suggested as antioxidants for lubricating oils. Whether or not such naphthenates are actually effective antioxidants under conditions of use in 40 internal combustion engines is, however, not a simple question to answer. The action of naphthenates in preventing or promoting oxidation appears to be a function of temperature to a very considerable extent. At atmospheric temperatures 45 an antioxidant effect may be observed, resulting in a decrease in the tendency of the compounded oil to form sludge on oxidation. At somewhat higher temperatures, however, metallic naphthenates such as copper naphthenate 50 may have exactly the opposite effect. We have found, for example, that copper naphthenate will actually increase sludge formation at a temperature of 310° F. when compounded with a well known Pennsylvania motor oil of SAE 20 55 grade. At still higher temperatures, of say from 350° to 600° F. or even higher, naphthenates tend to exert a pro-oxidant effect on petroleum oils, so strong as to cause the oil to oxidize fairly completely and leave a minimum of residue.

Since these metallic naphthenates in general do have such a pro-oxidant effect, it has been suggested that certain naphthenates, such as aluminum naphthenate and calcium naphthenate, 60 be used as anti-ring-sticking agents for lubricants, especially lubricants intended for use in Diesel and other heavy-duty internal combustion engines.

We have found, however, that nickel naphthenate, the use of which for the purpose indicated has not to our knowledge been suggested by any prior worker in the art, is exceptionally useful and advantageous, when incorporated in petroleum lubricating oils intended for use in internal combustion engines, in improving the 75

upper cylinder performance characteristics and reducing the ring-sticking tendencies of the oil, without on the other hand promoting oxidation under the conditions normally obtained in the 5 crankcases of internal combustion engines or otherwise harming the oil.

Not only have we found that far smaller amounts of nickel naphthenate are necessary for incorporation in lubricating oils in order to give 10 a desired degree of improvement than is true of other naphthenates, but we have also found that nickel naphthenate is effective in producing improvement of certain highly refined oils of the character set forth hereinabove, the upper cylinder 15 performance characteristics and ring-sticking tendencies of which are not substantially improved by the incorporation therein of other naphthenates, such as aluminum naphthenate.

20 In its preferred embodiment, therefore our invention comprises a lubricant for internal combustion engines, particularly of the heavy-duty type (Diesel and aircraft engines), comprising a major amount of a highly refined oil, such as 25 an oil obtained from a Pennsylvania crude or equivalent thereto, having a high viscosity index and a high inherent stability, and having incorporated therein a small amount of nickel naphthenate. The oil base is preferably a distillate 30 oil, although residual stocks may be employed when desired.

We have found, however, that the use of 35 nickel naphthenate is also advantageous with respect to other types of oils and to the lubrication of internal combustion engines generally, and therefore our invention in a broader aspect 40 also comprehends lubricants comprising various petroleum lubricating oils of the grades commonly used for all types of internal combustion 45 engines and having incorporated therein small amounts of nickel naphthenate.

Ordinarily the amount of nickel naphthenate thus employed will run from 0.05 to 2.0 per cent by weight of the lubricating oil base, the precise 50 amount depending upon the characteristics of the oil and the severity of the conditions to which the oil may be expected to be subjected. However, we have found that out of a large number 55 of compounded oils tested, the best results were achieved with respect to an aluminum-chloride-refined, non-residual Pennsylvania lubricating oil, of SAE 10 or 20 grade, containing 0.2 per cent of nickel naphthenate. This applies to Diesel-type engines primarily; for other engines, oils of different viscosities may be used.

This particular compounded oil has been found to be exceptionally advantageous and desirable. It has been subjected to a large number of tests 60 of different types, all indicative of the performance of the tested lubricant when used in internal combustion engines, and the results of such tests uniformly show improvement over the use of the uncompounded oil alone, as well as over the use of other oils when compounded 65 with the same addition agent and over the same or other oils when compounded with other addition agents including other types of metallic naphthenates.

The view has been expressed by some workers 70 in the art that metallic soaps such as aluminum naphthenate are effective in preventing ring-sticking and permitting freedom from deposition of undesirable solids in internal combustion engines because of a "detergent action," it being 75 postulated that such an agent assists in wash-

ing away or preventing the accumulation of deposits rather than by virtue of any action tending to prevent the initial formation of materials which if accumulated would form such deposits. While we do not desire to limit our 5 invention to any particular theory, nevertheless we are not in accord with the foregoing theory of detergent action and believe rather that the action of nickel naphthenate in the lubricant composition of our invention is primarily due 10 to the prevention in the first instance of any tendency to form gummy or lacquer-like residues. A detergent action may be incidental.

In support of our conclusions in this respect, we desire to refer to the results obtained in certain tests in which small strips of aluminum, coated with 20 per cent solutions in hexane of oils and compounded oils containing naphthenates were exposed to a temperature of 625° F. for 30 minutes in a gas-fired oven. Following 20 such exposure, the strips were examined for staining as an evidence of formation of gum or lacquer-like residues. A highly refined, paraffinic oil, when subjected to this test, produced a bad stain on the testing strips, indicating a 25 substantial deposit of lacquer-like material. The same oil, when compounded with 0.5 per cent of aluminum naphthenate, showed no improvement. The same oil when compounded with 0.5 per cent of calcium naphthenate showed 30 only a slight improvement, but staining was still evident. However, when the same oil was compounded with 0.5 per cent of nickel naphthenate and subjected to the foregoing test, no stain whatsoever was evident, the metal strips being 35 clean and bright after the test.

The lacquer and gum deposit or stains produced in the foregoing tests appear to be analogous to similar deposits formed on the piston rings and grooves during the operation of internal combustion engines and leading to ring-sticking. It appears likely that the efficacy of nickel naphthenate in preventing the formation of lacquer-like and gummy deposits in these tests is strictly analogous to the effect of nickel naphthenate in 45 preventing ring-sticking and deposition of gum and lacquer-like deposits on the pistons in engine tests, possibly on account of an acceleration of 50 oxidation of unvolatilized portions of the oil to the point of complete oxidation, thereby preventing the formation of intermediate products of oxidation of gum or lacquer-like nature.

We have carried out a number of engine tests for the purpose of comparing the compounded 55 oils of our invention with uncompounded oils and with oils compounded in the manner and according to the teachings of the prior art, with results uniformly indicating the superiority of the compounded oils of our invention.

In one group of engine tests, no fixed ring clearance was observed, some variation in the side clearance of the rings in the grooves (corresponding to manufacturing and replacement tolerances allowed by the engine manufacturer) being characteristic of the tests. This group of tests included individual tests covering 25 hour periods and 50 hour periods, respectively.

The data from the 25-hour tests in this group indicated clearly the effectiveness of 0.2 per cent 70 of nickel naphthenate, when added to a highly refined oil, in reducing ring-sticking, carbon and sludge deposition and in preventing lacquering of the piston surfaces. On the other hand, the average results of these 25-hour tests indicated 75 no improvement in engine performance resulting

from the addition of the same amount of aluminum naphthenate to the same oil.

In the 50-hour tests in this group, the data showed that a highly refined oil of the character indicated above, compounded with 0.2 per cent nickel naphthenate, was almost entirely free of any ring-sticking tendency, whereas under precisely the same conditions of testing the oil alone caused appreciable ring-sticking. Carbon and sludge deposition in the ring grooves and lacquering of the ring skirt were also lower for the compounded oil, and tests indicating the physical characteristics of the used oils after test showed a substantial improvement in quality with respect to the compounded oil, in comparison with the un compounded oil alone. These tests also indicated a substantial improvement in favor of the aforesaid compounded oil in comparison with an oil obtained from Coastal crude containing approximately 1.44 per cent of aluminum naphthenate.

One criticism which has been directed to the testing data obtained in reference to ring-sticking has been to the effect that certain anti-ring-sticking agents may owe their effectiveness to increased wear rather than to any inherent tendency to prevent formation of deposits known to cause ring-sticking. With this in mind, a second group of tests was formed in which an effort was made to eliminate, as far as possible, the effect of variation in ring clearance. In these tests the engine was disassembled and inspected at 25 hour intervals and any effect on ring-sticking produced by variation in ring clearance was eliminated by adjusting the side clearance in the grooves to a fixed value of 0.0015 inch around the circumference of each ring before each testing period. The results of this group of tests conformed to those of the previously mentioned group of tests, and demonstrated the marked superiority of an oil composition comprising an aluminum-chloride-refined Pennsylvania distillate oil compounded with 0.2 per cent of nickel naphthenate. This compounded oil caused less ring-sticking in 100 hours of testing than was caused by the oil alone in a 75 hour test period. Sludge deposition in the ring grooves and lacquering of the piston surfaces were also considerably lower in the case of the compounded oil for equivalent testing periods, and an examination of the used oils was also very much in favor of the compounded oil.

In this connection it may be noted, without attempting to pass any final opinion upon the effect of engine wear in the presence of metallic naphthenates, that there is ample theoretical reason for believing that nickel naphthenate has a far smaller tendency to promote wear than aluminum naphthenate, which has heretofore been regarded as among the best of the naphthenates for the particular problem with which we are concerned. Aluminum oxide (corundum), representing the ash produced by oxidation of aluminum naphthenate, is a much harder and more abrasive material than nickel oxide, which may be produced by the oxidation of nickel naphthenate. On this basis alone, it is reasonable to expect that nickel naphthenate does not have the pronounced abrading and wearing tendencies characteristic of aluminum naphthenate.

In addition to the foregoing tests, we have carried out competitive tests on a number of competitive oils which are now in common use for the lubrication of Diesel engines and which have been recommended by one of the manufacturers of these engines as superior Diesel engine oils. Examination of these oils shows that they are all low-viscosity Coastal oils compounded with aluminum or calcium soaps in amounts varying from 0.5 to 1.5 per cent. All of these oils proved to be definitely inferior to our preferred composition consisting of an aluminum-chloride-refined Pennsylvania distillate oil containing 0.2 per cent of nickel naphthenate.

It should be observed that while we believe that we are the first to suggest and demonstrate the remarkable effectiveness of nickel naphthenate as an addition agent in the compounding of oils for the purposes indicated, we do not claim that oils containing nickel naphthenate alone, particularly the more highly refined oils, are especially effective in meeting specific bearing-corrosion problems when encountered at high temperatures. However, a combination of nickel naphthenate and certain types of alkylated phenols has been found to be especially advantageous for this purpose. Oils containing such a combination of addition agents are described and claimed in the copending application of Oliver L. Brandes, filed concurrently herewith, Serial No. 251,416, now issued as Patent 2,202,826, of June 4, 1940, and constitute a specific improvement in the generic invention set forth herein.

While we have described our invention hereinabove with respect to various specific details and embodiments and particularly with reference to a preferred specific embodiment, it will be understood by those skilled in the art that our invention in its broadest aspect is not limited to such details, but may be variously practiced and embodied within the scope of the appended claims.

What we claim is:

1. An improved lubricant for use in internal combustion engines, comprising a major amount of a petroleum lubricating oil having incorporated therein a small amount of nickel naphthenate.

2. An improved lubricant for use in internal combustion engines, comprising a major amount of a petroleum lubricating oil having incorporated therein from 0.05 to 2.0 per cent of nickel naphthenate.

3. An improved lubricant for use in internal combustion engines, comprising a major amount of a highly refined and highly paraffinic petroleum lubricating oil, having a high viscosity index, and having incorporated therein a small amount, less than 2 per cent by weight, of nickel naphthenate.

4. The method of reducing ring-sticking tendencies in an internal combustion engine which comprises supplying to such engine, as a lubricant therefor, a petroleum lubricating oil having incorporated therein a small amount of nickel naphthenate.

NORBERT F. TOUSSAINT.  
HANNIBAL J. R. GASPARI.  
HENRY A. AMBROSE.